

1

3,020,235

## FERROMAGNETIC MATERIAL

Gerard Heinrich Jonker and Poul Bernard Braun, Eindhoven, Netherlands, assignors to North American Philips Company, Inc., New York, N.Y., a corporation of Delaware

No Drawing. Filed Oct. 14, 1957, Ser. No. 689,740  
Claims priority, application Netherlands Oct. 19, 1956  
5 Claims. (Cl. 252—62.5)

The ferromagnetic materials, according to the invention consist of crystals or mixed crystals of compounds having a chemical composition according to the formula

$\text{Ba}_{(1-a-b-c)} \text{Sr}_a \text{Pb}_b \text{Ca}_c \text{Me}^{\text{II}}_{(2-d-e-f)} \text{Co}^{\text{III}}_d \text{Cu}^{\text{I}}_e \text{Mn}^{\text{II}}_f \text{Fe}^{\text{III}}_{(3g-e)} \text{Co}^{\text{III}}_g \text{O}_{10}$

where  $\text{Me}^{\text{II}}$  represents at least one of the bivalent metals from the series comprising Fe, Ni, Zn and Mg and where

$$\begin{aligned} 0 \leq a &\leq 1.0 \\ 0 \leq b &\leq 0.7 \\ 0 \leq c &\leq 0.6 \\ 0 \leq d &\leq 2 \\ 0 \leq e &\leq 0.6 \\ 0 \leq f &\leq 0.6 \\ 0 \leq g &\leq 0.5 \end{aligned}$$

which compounds have a rhombohedral crystal structure the elementary cell of which can be described in the hexagonal crystal system by a  $c$ -axis of about 113.1 Å. and an  $a$ -axis of about 5.9 Å. A small part of ferric ions ( $\text{Fe}^{\text{III}}$ ) also can be replaced by trivalent chromium ( $\text{Cr}^{\text{III}}$ ) and aluminum ( $\text{Al}^{\text{III}}$ ) ions.

These materials have valuable electrical and magnetic properties. For example, they exhibit a saturation magnetisation of the same order of magnitude as the ferromagnetic ferrites having the crystal structure of the mineral spinel, the so-called "spinel structure." Like most of these ferrites, most of the materials in accordance with the invention have a high specific resistivity. Thus these materials can be fabricated into cores for use at high frequencies, in many cases at frequencies of 200 mc./sec. and more, since the high specific resistivity gives rise to small losses.

Unlike the ferromagnetic ferrites having a spinel structure, the initial permeability, for many of these materials is constant up to much higher frequencies. Since the use of ferromagnetic cores in a frequency range in which the initial permeability is not constant generally involves the occurrence of high electro-magnetic losses, the novel materials can be used as ferromagnetic bodies up to the above-mentioned higher frequencies in all cases where low electro-magnetic losses are required.

In ferromagnetic materials of hexagonal crystal structure, the crystal anisotropy is given as a first approximation by the expression

$$F_K = K_1' \sin^2 \theta$$

(see R. Becker and W. Doring, "Ferromagnetismus," 1939, page 114). If  $K_1'$  is positive (so-called "positive" crystal anisotropy), the hexagonal axis of the crystal is the preferred direction of magnetisation. If, however,  $K_1'$  is negative (which condition will hereafter be referred to as "negative" crystal anisotropy), this means that the spontaneous magnetisation is directed at right angles to the hexagonal axis and consequently parallel to the basal plane of the crystal. In the latter case, the crystal has a so-called "preferred plane" of magnetisation (there may, however, still be a comparatively weak preference of the magnetisation for certain directions in the basal plane). In part of the novel materials under consideration,  $K_1'$  is negative. In this event, in each crystal the direction of the spontaneous magnetisation lies in the basal plane and in this plane the direction of magnetisation is more read-

2

ily rotatable than in a direction which does not lie in this plane. In these materials, the initial permeability has values which are high enough to be of interest for electro-mechanical use. This initial permeability is constant up to a far higher frequency than in ferromagnetic ferrites of spinel structure having an equal value of the initial permeability at low frequency. The materials in accordance with the invention having positive crystal anisotropy offer novel possibilities of manufacturing, for example, ferro-magnetic bodies having permanent magnetic properties and ferro-magnetic bodies for use in microwave-apparatus.

In order to determine whether or not crystals having a preferred direction of magnetisation or crystals having a preferred plane of magnetisation are involved, use may be made of the following identifications test:

A small amount, for example 25 mgs., of the crystal material to be examined is mixed as a fine powder with a few drops of a solution of an organic binder or adhesive in acetone, the mixture being spread on a glass slide. This slide is arranged between the poles of an electromagnet so that the lines of magnetic force are at right angles to the surface of the slide. By gradually increasing the electric direct current of the electromagnet, the magnetic field strength is increased, so that the powder particles rotate in the field in a manner such that either the preferred direction of the magnetisation or the preferred plane of the magnetisation becomes substantially parallel to the direction of the lines of magnetic force. By proceeding carefully, a coagulation of the powder particles can be avoided. After evaporation of the acetone, the powder particles adhere to the glass surface in a magnetically orientated condition. By means of radiographs it can now be determined which orientation of the powder particles has been produced by the action of the magnetic field. This can be effected, for example, with the aid of an X-ray diffractometer (for example, an apparatus as described in "Philips' Technical Review," 16, pages 123-133, 1954-1955). An increased occurrence of the reflections at planes at right angles to the hexagonal  $c$ -axis (so-called "001-reflections") being observed in the case of a preferred direction parallel to the  $c$ -axis as compared with a radiograph of a nonoriented specimen. In the case of a preferred plane at right angles to the hexagonal  $c$ -axis, an increased occurrence of reflections at planes parallel to this  $c$ -axis (so-called " $hk0$ -reflections") is observed.

The crystal anisotropy constant  $K_1'$  depends upon the chemical composition and also for each material, upon the temperature. In many of the novel materials under consideration a temperature can be determined below which the crystal anisotropy is negative and above which it is positive. The temperature of the reversing point of the crystal anisotropy depends mainly upon the content of bivalent cobalt. The reversal point lies at room temperature, if the material contains a certain amount of Co, which amount slightly depends upon the other small bivalent ions but is about  $\frac{1}{3}$  of the total amount of small bivalent ions. If more than about  $\frac{1}{3}$  of the small bivalent ions is Co ( $d$  greater than or about equal to 0.6), the crystals of the materials have a preferred plane of the magnetisation at room temperature. If less than about  $\frac{1}{3}$  of the small bivalent ions is Co, ( $d$  is less than or about equal to 0.6), the crystals of the materials have a preferred direction of the magnetisation at room temperature. Obviously, the choice of the material is determined by the fact whether a positive or a negative crystal anisotropy is desired within the operating range.

It has been found that in materials which have a negative crystal anisotropy constant and consequently a preferred plane of the magnetisation, the value of the initial permeability can be further increased if in the formula

ferric-ions are partly replaced by trivalent Co-ions, but this is only possible to about 1.5 atomic percent expressed by  $0.2 \leq g \leq 0.5$ . Comparatively high values of the initial permeability are also found in the materials containing Fe as the bivalent metal; however, these materials naturally have a low specific resistivity which involves the production of eddy-current losses at high frequencies.

The production of the materials according to the invention is preferably effected by heating (sintering) a finely powdered mixture of the component metal oxides of the novel compounds in about correct proportions. Obviously, at least one of the component metal oxides can be wholly or partially replaced by compounds which can be converted into metal oxides by heating, for example carbonates, oxalates and acetates. The component metal oxides can also be wholly or partially replaced by one or more reaction products of at least two of the component metal oxides, for example  $\text{BaFe}_{12}\text{O}_{19}$ . The term "correct proportions" as used herein is to be understood to mean proportions of the amounts of the metals in the initial mixture equal to those in the materials to be produced. When using this method of producing the materials in accordance with the invention, the materials which do not contain Sr, Pb or Ca are produced by far the most readily.

If desired, the finely powdered initial material may be presintered, the reaction product being ground again and the powder thus obtained being re-sintered, and this sequence of operations may be repeated once or several times. This method of sintering is known per se, for example in the production of ferro-magnetic ferrites having spinel structure (see for example J. J. Went and E. W. Gorter, "Philips Technical Review," 13, page 183, 1951-1952). The temperature of the sintering or final sintering process is between about 1000° C. and about 1450° C., preferably between 1200° C. and 1350° C.

In order to promote the sintering process, sintering agents, for example silicates and fluorides, may be added. Bodies consisting of the above-described ferromagnetic materials can be formed either by immediately sintering the initial mixture of the metal oxides or the like in the desired shape or by pulverizing the reaction product of the presintering process and shaping it, if required after the addition of a binder, into the desired form, after which it may be re-sintered or hardened.

By sintering at a temperature materially exceeding 1200° C. and/or by sintering in a gas-atmosphere containing comparatively little oxygen, a material can be produced having a comparatively high proportion of  $\text{Fe}^{II}$ , so that the specific resistivity can be reduced to values of less than 10 ohm-cm. If this is not desired, because the material is to be used in magnetic cores for use at high frequencies without the production of excessive eddy-current losses at those frequencies, excessive formation of ferrous ions must be avoided or any excessive amount of ferrous ions must subsequently be oxidized to ferric ions in known manner, for example by heating again in oxygen at a temperature between 1000° C. and 1250° C.

In producing the materials in accordance with the invention which contain lead, special precautions must be taken. Part of the  $\text{PbO}$  escapes from the product during heating due to its volatility, so that it is desirable for the initial mixture to contain an amount of lead in excess of the proportions of the metals in the material to be produced.

As is usual, the electromagnetic losses are indicated by a loss factor  $\tan \delta = \mu''/\mu'$  (see J. Smit and H. P. J. Wijn "Advances in electronics," VI, 1954, page 69, formula No. 37). The quantity  $\mu'$  is the so-called "real" part of the initial permeability. This property and  $\tan \delta$  will be given as numerical values in the following examples.

#### EXAMPLE I

A mixture of  $\text{BaCO}_3$ ,  $\text{CoCO}_3$  and  $\text{Fe}_2\text{O}_3$  in proportions of 2 mols of  $\text{BaCO}_3$ , 1 mol of  $\text{CoCO}_3$  and 9 mols

of  $\text{Fe}_2\text{O}_3$ , which corresponds to the desired compound  $\text{Ba}_4\text{Co}_2\text{Fe}_{36}\text{O}_{60}$  was mixed with ethyl-alcohol in a ball mill for half an hour. After drying, the mixture was pre-fired in air at 1000° C. for 15 hours, and the reaction product then ground together with ethyl alcohol in a ball mill for 1 hour. After drying, a small amount of a solution of an organic binder was added to the product and part of this mixture was compressed into a tablet which was fired in oxygen at 1260° C. for 1 hour.

In like manner, tablets were produced from mixtures comprising, in addition to  $\text{BaCO}_3$  and  $\text{Fe}_2\text{O}_3$ ,  $\text{CoCO}_3$  and  $\text{MgO}$ ,  $\text{CoCO}_3$  and  $\text{MgO}$ ,  $\text{MgO}$ ,  $\text{NiO}$  and  $\text{ZnO}$ , respectively in a ratio of 2 mols of  $\text{BaCO}_3$  and 9 mols of  $\text{Fe}_2\text{O}_3$  to 0.5 mol of  $\text{CoCO}_3$  and 0.5 mol of  $\text{MgO}$ , 0.25 mol of  $\text{CoCO}_3$  and 0.75 mol of  $\text{MgO}$ , 1 mol of  $\text{MgO}$ , 1 mol of  $\text{NiO}$  and 1 mol of  $\text{ZnO}$ , respectively, corresponding to the desired compounds  $\text{Ba}_4\text{CoMgFe}_{36}\text{O}_{60}$ ,  $\text{Ba}_4\text{Co}_{0.5}\text{Mg}_{1.5}\text{Fe}_{36}\text{O}_{60}$ ,  $\text{Ba}_4\text{Mg}_2\text{Fe}_{36}\text{O}_{60}$ ,  $\text{Ba}_4\text{Ni}_2\text{Fe}_{36}\text{O}_{60}$  and  $\text{Ba}_4\text{Zn}_2\text{Fe}_{36}\text{O}_{60}$ , respectively.

Finally, a mixture of  $\text{BaCO}_3$ ,  $\text{ZnO}$  and  $\text{Fe}_2\text{O}_3$  in a ratio of 2 mols of  $\text{BaCO}_3$ , 0.75 mol of  $\text{ZnO}$  and 9.125 mol of  $\text{Fe}_2\text{O}_3$ , which corresponds to the desired compound



was prepared, pre-fired and ground in the above described manner. A tablet was pressed from this mixture and fired at 1300° C. in technical nitrogen for 1 hour.

Examination by means of X-rays showed that the reaction product consisted substantially entirely of crystals having the desired structure. The saturation magnetisation of all these materials exceeded 2000 gauss. The sign of the crystal anisotropy at room temperature was also determined by X-ray examination of the materials in the manner referred to hereinbefore. The results are shown in Table I. In this and the following tables the column captioned "main constituent" denotes chemical formulae which were deduced from the composition of the initial mixtures and from the X-ray examination.

#### Table No. I

Crystal anisotropy at room temperature of a number of materials according to the invention.

| Main constituent:                                                                   | Sign of the crystal anisotropy |
|-------------------------------------------------------------------------------------|--------------------------------|
| $\text{Ba}_4\text{Co}_2\text{Fe}_{36}\text{O}_{60}$                                 | —                              |
| $\text{Ba}_4\text{CoMgFe}_{36}\text{O}_{60}$                                        | —                              |
| $\text{Ba}_4\text{Co}_{0.5}\text{Mg}_{1.5}\text{Fe}_{36}\text{O}_{60}$              | +                              |
| $\text{Ba}_4\text{Mg}_2\text{Fe}_{36}\text{O}_{60}$                                 | +                              |
| $\text{Ba}_4\text{Ni}_2\text{Fe}_{36}\text{O}_{60}$                                 | +                              |
| $\text{Ba}_4\text{Zn}_2\text{Fe}_{36}\text{O}_{60}$                                 | +                              |
| $\text{Ba}_4\text{Zn}_{1.5}\text{Fe}_{6.5}\text{Fe}^{\text{III}}_{36}\text{O}_{60}$ | +                              |

#### EXAMPLE II

A mixture of  $\text{BaCO}_3$ ,  $\text{CoCO}_3$  and  $\text{Fe}_2\text{O}_3$  in a ratio according to the formula  $\text{Ba}_4\text{Co}_2\text{Fe}_{36}\text{O}_{60}$  was mixed with ethyl alcohol in a ball mill for half an hour and subsequently pre-fired in air at 1000° C. for 15 hours. The reaction product was ground together with ethyl alcohol in a ball mill for 1 hour and after drying and the addition of a small amount of an organic binder the product was compressed to form rings. One ring was fired in air at 1280° C. for 1 hour and subsequently slowly cooled in air. The properties of this ring are given in Table 2 under 1. Another ring was fired in oxygen at 1270° C. for 3 hours. The properties of this ring are given in Table 2 under 2. A third ring was fired in oxygen at 1270° C. for three hours, cooled at room temperature and subsequently heated again in oxygen at 1180° C. for 4 hours. The properties of this third ring are given in Table 2 under 3. Examination by means of X-rays showed that all the reaction products consist entirely of crystals having the desired structure. The measurements given in this and the following tables were obtained from rings in the demagnetised condition at room temperature according to the method described by C. M. van der Burgt, M. Gevers and H. P. J. Wijn in

"Philips Technical Review," 14 pages 246-252 (1952-1953).

In Table 2 and the following tables, columns designated  $\Omega$ -cm.,  $\mu'$  and  $\tan \delta$  designate specific resistivity, initial (real) permeability and loss factor, respectively, at room temperature of the materials according to the invention. Initial permeability and loss factor were also measured at frequencies of 10 kc./sec., 80 mc./sec., 260 mc./sec. and 500 mc./sec.

Table 2

| No.    | Main constituent        | $\Omega$ -cm. | 10 kc./s. |        | 80 mc./s. |               | 260 mc./s. |        | 500 mc./s. |               |
|--------|-------------------------|---------------|-----------|--------|-----------|---------------|------------|--------|------------|---------------|
|        |                         |               | $\mu'$    | $\mu'$ | $\mu'$    | $\tan \delta$ | $\mu'$     | $\mu'$ | $\mu'$     | $\tan \delta$ |
| 1..... | $Ba_4Co_2Fe_{35}O_{60}$ | $10^3$        | 4.7       | 4.4    | 0.05      |               | 4.3        | 0.14   | 4.3        | 0.25          |
| 2..... | $Ba_4Co_2Fe_{35}O_{60}$ | $10^7$        | 3.1       | 2.7    | 0.01      |               | 2.9        | 0.07   | 2.9        | 0.19          |
| 3..... | $Ba_4Co_2Fe_{35}O_{60}$ | $>10^7$       | 3.8       | 3.1    | $<0.01$   |               | 3.3        | 0.04   | 3.5        | 0.24          |

## EXAMPLE III

A mixture of  $BaCO_3$ ,  $CoCO_3$  and  $Fe_2O_3$  in a ratio corresponding to the formula  $Ba_4Co_2Fe_{35}O_{60}$  was mixed with ethyl alcohol in a ball mill for half an hour. After drying and the addition of a small amount of an organic binder, part of the product was compressed into a ring and fired in oxygen at  $1260^\circ C$ . for 1 hour. The ring was subsequently cooled to room temperature and again heated in oxygen at  $1180^\circ C$ . for 4 hours. In the same manner, rings were produced from mixtures of  $BaCO_3$ ,  $CoCO_3$ , and  $Fe_2O_3$  in ratios corresponding to the formulas



and



X-ray examination showed that all the reaction products

A mixture of  $BaCO_3$ ,  $CoCO_3$  and  $Fe_2O_3$  in a ratio corresponding to the formula

5



was mixed with ethyl alcohol in a ball mill for half an hour and subsequently prefired in air at  $1000^\circ C$ . for 15 hours. The reaction product was ground with ethyl

## EXAMPLE IV

alcohol in a ball mill for 1 hour and, after drying and the addition of a small amount of an organic binder, rings were pressed from the product. One ring was fired in air at  $1280^\circ C$ . for 3 hours. The properties of this ring are listed in Table 4 under 1. Another ring was fired in air at  $1280^\circ C$ . for 3 hours, cooled to room temperature and subsequently heated again in oxygen at  $1100^\circ C$ . for 4 hours. The properties of this ring are listed under 2 in Table 4. A third ring, pressed from the ground, not prefired starting mixture was fired in oxygen at  $1260^\circ C$ . for 1 hour, subsequently cooled to room temperature and again heated in oxygen at  $1180^\circ C$ . for 4 hours. Finally it was cooled in oxygen to room temperature. The properties of this ring are listed under 3 in Table 4. X-ray examination revealed that all the reaction products consisted entirely of crystals having the desired structure.

25

30

35

Table 4

| No.    | Main constituent                         | $\Omega$ -cm. | 10 kc./s. |        | 80 mc./s. |               | 260 mc./s. |        | 500 mc./s. |               |
|--------|------------------------------------------|---------------|-----------|--------|-----------|---------------|------------|--------|------------|---------------|
|        |                                          |               | $\mu'$    | $\mu'$ | $\mu'$    | $\tan \delta$ | $\mu'$     | $\mu'$ | $\mu'$     | $\tan \delta$ |
| 1..... | $Ba_4Co_2^{II}Fe_{35.5}Co_0^{III}O_{60}$ | $3.10^2$      | 11.5      | 10.4   | 0.10      |               | 9.2        | 0.26   | 8.3        | 0.60          |
| 2..... | $Ba_4Co_2^{II}Fe_{35.7}Co_0^{III}O_{60}$ | $5.10^4$      | 7.2       | 6.7    | 0.06      |               | 6.8        | 0.10   | 6.6        | 0.26          |
| 3..... | $Ba_4Co_2^{II}Fe_{35.5}Co_0^{III}O_{60}$ | $>10^7$       | 3.7       | 3.3    | $<0.01$   |               | 3.6        | 0.04   | 3.8        | 0.25          |

consisted entirely of crystals having the desired structure.

Furthermore a ring was produced in the manner described hereinbefore from a mixture of  $BaCO_3$ ,  $CoCO_3$  and  $Fe_2O_3$  in a ratio according to the formula



55

and this ring was shown by X-ray examination to consist substantially entirely of crystals having the desired structure.

The specific resistivity of all these products exceeds  $10^7$  ohm/cm. Further properties of these rings are given in Table 3.

Table 3

| Main constituent                         | 10 kc./s. |        | 80 mc./s. |        | 260 mc./s. |        | 500 mc./s. |        |
|------------------------------------------|-----------|--------|-----------|--------|------------|--------|------------|--------|
|                                          | $\mu'$    | $\mu'$ | $\mu'$    | $\mu'$ | $\mu'$     | $\mu'$ | $\mu'$     | $\mu'$ |
| $Ba_4Co_2Fe_{35}O_{60}$                  | 3.8       | 3.1    | $<0.01$   | 3.3    | 0.04       | 3.5    | 0.24       |        |
| $Ba_4Co_2^{II}Fe_{35.5}Co_0^{III}O_{60}$ | 3.7       | 3.3    | $<0.01$   | 3.6    | 0.04       | 3.8    | 0.25       |        |
| $Ba_4Co_2^{II}Fe_{35.7}Co_0^{III}O_{60}$ | 4.8       | 4.3    | $<0.01$   | 4.4    | 0.04       | 4.6    | 0.28       |        |
| $Ba_4Co_2^{II}Fe_{35.5}Co_0^{III}O_{60}$ | 4.9       | 4.4    | 0.01      | 4.4    | 0.04       | 5.1    | 0.22       |        |

## EXAMPLE V

A mixture of  $BaCO_3$ ,  $CoCO_3$  and  $Fe_2O_3$  in a ratio corresponding to the formula



60

was mixed with ethyl alcohol in a ball mill for half an hour. After drying, a small amount of an organic binder was added to the product, part of which was compressed to form a ring which was fired in oxygen at  $1260^\circ C$ . for 2 hours and subsequently slowly cooled in oxygen. By the same method rings were produced from mixtures

of  $\text{BaCO}_3$ ,  $\text{Fe}_2\text{O}_3$ ,  $\text{CoCO}_3$  and one of the compounds  $\text{ZnO}$ ,  $\text{MgCO}_3$ ,  $\text{NiO}$ ,  $\text{MnCO}_3$  and  $\text{CuO}$ , respectively, in ratios according to the formula:



X-ray examination showed that the reaction products consisted entirely of crystals having the desired structure. The properties of the rings are given in Table 5.

Table 5

| Main constituent                                                                                                 | 10 kc./s. |       |               | 80 mc./s. |       |               | 260 mc./s. |       |               | 500 mc./s. |       |               |
|------------------------------------------------------------------------------------------------------------------|-----------|-------|---------------|-----------|-------|---------------|------------|-------|---------------|------------|-------|---------------|
|                                                                                                                  | $\mu'$    | $\mu$ | $\tan \delta$ | $\mu'$    | $\mu$ | $\tan \delta$ | $\mu'$     | $\mu$ | $\tan \delta$ | $\mu'$     | $\mu$ | $\tan \delta$ |
| $\text{Ba}_4\text{Co}_{1.2}^{\text{II}}\text{Fe}_{35.5}\text{Co}_{0.5}^{\text{III}}\text{O}_{60}$                | 5.5       | 5.3   | 0.03          | 5.2       | 0.06  | 5.3           | 0.15       |       |               |            |       |               |
| $\text{Ba}_4\text{Co}_{1.2}^{\text{II}}\text{Zn}_{0.8}\text{Fe}_{35.5}\text{Co}_{0.5}^{\text{III}}\text{O}_{60}$ | 6.0       | 6.7   | 0.03          | 6.8       | 0.14  | 6.4           | 0.51       |       |               |            |       |               |
| $\text{Ba}_4\text{Co}_{1.2}^{\text{II}}\text{Mg}_{0.8}\text{Fe}_{35.5}\text{Co}_{0.5}^{\text{III}}\text{O}_{60}$ | 5.3       | 5.0   | 0.06          | 4.8       | 0.14  | 4.5           | 0.26       |       |               |            |       |               |
| $\text{Ba}_4\text{Co}_{1.2}^{\text{II}}\text{Ni}_{0.8}\text{Fe}_{35.5}\text{Co}_{0.5}^{\text{III}}\text{O}_{60}$ | 5.3       | 5.2   | 0.03          | 5.5       | 0.18  | 4.7           | 0.50       |       |               |            |       |               |
| $\text{Ba}_4\text{Co}_{1.0}^{\text{II}}\text{Mn}_{0.4}\text{Fe}_{35.5}\text{Co}_{0.5}^{\text{III}}\text{O}_{60}$ | 4.0       | 3.6   | <0.01         | 3.6       | 0.04  | 3.8           | 0.16       |       |               |            |       |               |
| $\text{Ba}_4\text{Co}_{1.0}^{\text{II}}\text{Cu}_{0.4}\text{Fe}_{35.5}\text{Co}_{0.5}^{\text{III}}\text{O}_{60}$ | 3.4       | 3.0   | <0.01         | 3.1       | 0.04  | 3.1           | 0.20       |       |               |            |       |               |

## EXAMPLE VI

The compounds  $\text{Ba}_{0.8}\text{Sr}_{0.2}\text{Fe}_{12}\text{O}_{19}$ ,  $\text{Ba}_{0.65}\text{Pb}_{0.15}\text{Fe}_{12}\text{O}_{19}$  and  $\text{Ba}_{0.85}\text{Ca}_{0.15}\text{Fe}_{12}\text{O}_{19}$  were produced by heating mixtures of  $\text{BaCO}_3$ ,  $\text{Fe}_2\text{O}_3$  and one of the compounds  $\text{SrCO}_3$ ,  $\text{PbCO}_3$  and  $\text{CaCO}_3$ , respectively, in ratios corresponding to those compounds at  $1000^\circ\text{C}$ . for 15 hours. From these compounds and  $\text{BaCO}_3$ ,  $\text{CoCO}_3$  and  $\text{ZnO}$ , mixtures were made in ratios of 3 mols of (Pa, Sr, Pb, Ba) $1\text{Fe}_{12}\text{O}_{19}$ , 1 mol of  $\text{BaCO}_3$ , 1.5 mol of  $\text{CoCO}_3$  and 0.5 mol of  $\text{ZnO}$ , corresponding to the desired compounds



and



To the mixture containing lead, 5% by weight of  $\text{PbCO}_3$  was added. The mixtures were ground with ethyl alcohol in a ball mill for 1 hour. After drying and the addition of a small amount of a solution of an organic binder, rings were pressed from the products, which were fired at  $1260^\circ\text{C}$ . in oxygen for 1 hour with the exception of the ring containing lead, which is fired at  $1240^\circ\text{C}$ . in oxygen for 1 hour. The properties of the rings are listed in Table 6.

Table 6

| Main constituent                                                                            | 10 kc./s. |       |               | 80 mc./s. |       |               | 260 mc./s. |       |               | 500 mc./s. |       |               |
|---------------------------------------------------------------------------------------------|-----------|-------|---------------|-----------|-------|---------------|------------|-------|---------------|------------|-------|---------------|
|                                                                                             | $\mu'$    | $\mu$ | $\tan \delta$ | $\mu'$    | $\mu$ | $\tan \delta$ | $\mu'$     | $\mu$ | $\tan \delta$ | $\mu'$     | $\mu$ | $\tan \delta$ |
| $\text{Ba}_{3.4}\text{Sr}_{0.6}\text{Co}_{1.5}\text{Zn}_{0.5}\text{Fe}_{36}\text{O}_{60}$   | 6.8       | 6.3   | 0.05          | 6.7       | 0.13  | 6.5           | 0.44       |       |               |            |       |               |
| $\text{Ba}_{3.55}\text{Pb}_{0.15}\text{Co}_{1.5}\text{Zn}_{0.5}\text{Fe}_{36}\text{O}_{60}$ | 3.8       | 3.4   | 0.04          | 3.5       | 0.13  | 3.2           | 0.33       |       |               |            |       |               |
| $\text{Ba}_{3.55}\text{Ca}_{0.45}\text{Co}_{1.5}\text{Zn}_{0.5}\text{Fe}_{36}\text{O}_{60}$ | 2.7       | 2.5   | 0.01          | 2.6       | 0.10  | 2.5           | 0.28       |       |               |            |       |               |

While we have thus described our invention in connection with specific examples and applications thereof we do not wish to be limited thereto as other embodiments will be readily apparent to those skilled in this art. The invention is defined in the appended claims which should be as liberally construed as permissible in view of the art.

What is claimed is:

1. A ferromagnetic material consisting essentially of crystals having the composition:



in which  $\text{Me}^{\text{II}}$  is at least one bivalent metal selected from the group consisting of  $\text{Fe}^{\text{II}}$ ,  $\text{Ni}$ ,  $\text{Zn}$  and  $\text{Mg}$  and in which

$a$  is at most 1,  $b$  is at most 0.7,  $c$  is at most 0.6,  $d$  is at most 2,  $e$  is at most 0.6,  $f$  is at most 0.6,  $g$  is at most 0.5, said crystals having a rhombohedral structure, the elementary cell of which can be described in the hexagonal crystal system by a  $c$ -axis of about 113.1 Å, and an  $a$ -axis of about 5.9 Å.

2. A ferromagnetic material consisting essentially of crystals having the composition:



in which  $\text{Me}^{\text{II}}$  is at least one bivalent metal selected from the group consisting of  $\text{Fe}^{\text{II}}$ ,  $\text{Ni}$ ,  $\text{Zn}$  and  $\text{Mg}$  and in which

$a$  is at most 1,  $b$  is at most 0.7,  $c$  is at most 0.6,  $d$  is at most 2,  $e$  is at most 0.6,  $f$  is at most 0.6,  $g$  is at most 0.5, said crystals having a rhombohedral structure, the elementary cell of which can be described in the hexagonal crystal system by a  $c$ -axis of about 113.1 Å, and an  $a$ -axis of about 5.9 Å, said crystals having at room temperature a preferred plane of magnetization.

3. A ferromagnetic material consisting essentially of crystals having the composition:



in which  $\text{Me}^{\text{II}}$  is at least one bivalent metal selected from the group consisting of  $\text{Fe}^{\text{II}}$ ,  $\text{Ni}$ ,  $\text{Zn}$  and  $\text{Mg}$  and in which  $a$  is at most 1,  $b$  is at most 0.7,  $c$  is at most 0.6,  $d$  is at least about 0.6 and at most 2,  $e$  is at most 0.6,  $f$  is at most 0.6,  $g$  is at least 0.2 and at most 0.5, said crystals having a rhombohedral structure, the elementary cell of which can be described in the hexagonal crystal system by a  $c$ -axis of about 113.1 Å, and an  $a$ -axis of about 5.9 Å.

4. A ferromagnetic material consisting essentially of crystals having the composition:



in which  $\text{Me}^{\text{II}}$  is at least one bivalent metal selected from the group consisting of  $\text{Fe}^{\text{II}}$ ,  $\text{Ni}$ ,  $\text{Zn}$  and  $\text{Mg}$  and in which  $a$  is at most 1,  $b$  is at most 0.7,  $c$  is at most 0.6,  $d$  is at most 0.6,  $e$  is at most 0.6,  $f$  is at most 0.6,  $g$  is at most 0.5, said crystals having a rhombohedral structure, the elementary cell of which can be described in the hexagonal crystal system by a  $c$ -axis of about 113.1 Å, and an  $a$ -axis of about 5.9 Å, said crystals having at room temperature a preferred direction of magnetization.

5. A ferromagnetic material consisting essentially of crystals having the composition:



in which  $\text{Me}^{\text{II}}$  is at least one bivalent metal selected from the group consisting of  $\text{Fe}^{\text{II}}$ ,  $\text{Ni}$ ,  $\text{Zn}$  and  $\text{Mg}$  and in which

in which  $Me^{II}$  is at least one bivalent metal selected from the group consisting of  $Fe^{II}$ , Ni, Zn and Mg and in which  $a$  is at most 1,  $b$  is at most 0.7,  $c$  is at most 0.6,  $d$  is at most about 0.6,  $e$  is at most 0.6,  $f$  is at most 0.6,  $g$  is at most 0.5, said crystals having a rhombohedral structure, the elementary cell of which can be described in the hexagonal crystal system by a  $c$ -axis of about 113.1 Å., and an  $a$ -axis of about 5.9 Å., said crystals having at room temperature a preferred direction of magnetization.

References Cited in the file of this patent

UNITED STATES PATENTS

- |           |                      |                |
|-----------|----------------------|----------------|
| 2,736,708 | Crowley et al. ----- | Feb. 28, 1956  |
| 2,762,777 | Went et al. -----    | Sept. 11, 1956 |
| 2,778,803 | Crowley -----        | Jan. 22, 1957  |

10 5 165,447

FOREIGN PATENTS

- |                     |               |
|---------------------|---------------|
| Netherlands -----   | Aug. 15, 1955 |
| Great Britain ----- | Nov. 28, 1951 |
| Great Britain ----- | July 4, 1956  |
| Australia -----     | Oct. 4, 1955  |

OTHER REFERENCES

- Snoek: *Physica*, June 1936, page 481.  
 Jonker et al.: *Philips Tech. Rev.*, Nov. 30, 1956, pp. 145-153.  
 Went et al.: *Philips Tech. Rev.*, January 1952, p. 197.  
 Bazorth: *Physical Rev.*, Sept. 15, 1955, pp. 1788-1798.  
*J. of the Institute of Electrical Engineers, Japan*, November 1937, pp. 3, 5, 7.